

## UNITED STATES PATENT OFFICE

2,321,227

## ALLOY

William C. McLott, Grand Rapids, Mich.

No Drawing. Application August 6, 1941,  
Serial No. 405,627

4 Claims. (Cl. 75—125)

This invention relates to a new alloy of which the principal ingredients are iron, chromium, molybdenum and copper with small amounts of titanium and manganese, carbon and silicon. The alloy may be used in the form of a weld rod in oxyacetylene and electric welding. In connection with electric welding, because of the very high temperatures produced a special and novel flux must be used and my invention is concerned not only with the metallic alloy but also with the flux required in the electric welding or deposition of the metal alloy.

In the alloy which I have produced the chromium and molybdenum used provide an exceptionally tough bond, which is three or four times greater than the best high test steels to hold the copper in minute crystalline structure in the alloy. The copper converts to a hexagonal crystal of an extremely small size which is much harder and tougher than practically any known synthetic substance and which crystals do not melt in passing through the electric arc.

The alloy combination when melted and deposited properly onto a prepared surface is bonded thereto by a small amount of the chromium and molybdenum of the melted alloy uniting with the base metal, producing a very strong bond which holds the very hard alloy upon the base in a better and superior manner to anything which I have previously known. The alloy is not designed to serve as a cutting edge for metal turning but holds an edge well for rock cutting, food chopping or other places where a keen edge is not required, for example on axes and various types of cutting knives such as those cutting ensilage and the like. The alloy may be readily applied to gray cast iron or to any steel base depositing thereon in either a single layer or in successive layers. A good flux to clean oxide from the surface of the base is requisite in order for the alloy to unite with and form a tough bond.

The alloy which I have produced possesses an affinity for tungsten carbide adhering thereto with great strength so that it can be removed only by grinding or oxidizing at high temperatures. This makes it valuable for the setting of carbide inserts to fishtail bits and core bits in rock drilling such as in drilling oil wells and in mining operations. It also may be applied to parts which are subsequently to be carbonized or nitrided. The specific gravity of the alloy is substantially the same as that of steel so that it does not bury itself by gravity in molten steel or in the molten surface of a steel base when applied thereto.

I have found that any alloy composed of chromium of approximately 25 to 33%, molybdenum 1.5% to 5%, copper 1 to 3%, manganese 0.5 to 2%, titanium 0.3 to 1.5% with carbon 3 to 3.25% and silicon 0.7 to 1.3%, the balance being of iron produces an alloy which is very hard and resistant to abrasion; has a high strength and which can be deposited either by oxy-acetylene or electric arc melting. The metal thus deposited has a hardness from 610 to 650 Brinell, the lower degrees of hardness being that when deposited and bonded to a mild or tool steel base and the higher degrees when deposited on bases of high alloy or manganese steels. The tensile strength ranges from 90,000 to 110,000 pounds per square inch. Its resistance to abrasion as compared to that of the diamond is as 79 to 100. The melting point is approximately 2400° F., its specific gravity is substantially 8.3. There is no elongation at temperatures under 1800° F. and scarcely and at the worst but a very slight elongation at temperatures over 1800° F. Succeeding deposits of the alloy may be laid one upon another without removal of a previous or old deposit, this being an advantage in the repair of previous deposits or overlays.

The titanium used accelerates the proper relation of the chromium, iron and carbon with an increase in the production of iron chrome carbide. The manganese to and including 0.5% is used to control sulphur and phosphorus and that used above 0.5% acts to cause the formation of a Penta carbide of chrome iron.

The alloy in the form of rods may be used without any flux coating in the oxy-acetylene melting of the rods and their deposition upon a base. The temperature of the melting flame will not exceed 3500° F. and it is only when temperatures reach 3600° F. and more that there are carbon and nitrogen metallic troubles, that is, the alloy when subjected to a temperature exceeding 3600° F. in the presence of air which contains a large proportion of nitrogen is detrimentally affected by nitrogen combining with the chromium and iron.

For the alloy rods for use in electric melting I have developed a novel flux. This flux for its dry elements comprises marble 38 to 42%, graphite 35 to 38%, fluorspar 15 to 18%, titanium, 6 to 8%; and when the smaller percentages are used any balance required to make the full 100% is of a diatomaceous earth. The liquid elements used are sodium silicate 30% and distilled water 70%.

65 The liquid and dry elements are mixed together

in proportions of 55% of dry elements to 45% of wet elements.

In applying the flux coating to the rods the amount used is such that the dry element weight of the flux approximates 6% of the total weight of the rod while the metallic alloy consists of the remaining 94% of the weight.

The marble, graphite and fluorspar and a diatomaceous earth provide the oxygen exclusion feature of the flux while the titanium in the flux insures against the detrimental effects of nitrogen in the air combining with elements of the alloy composition to the detriment of the deposit.

The present alloy may be readily welded on steel of any carbon content and on cast iron and all types of alloy steels. The phosphorus and sulphur which may be present in very small amounts because unavoidable are counteracted as to their effect by use of manganese, and copper in its minute crystalline form provides an extremely hard and tough constituent which is not affected as to its properties when subjected to the high temperatures present in electric melting and depositing of the metal.

The most essential components of the alloy in addition to the iron are the chromium, molybdenum and copper. The carbon and silicon are in proper balance, the manganese need only be used in the amount to control the phosphorus and sulphur, but the alloy is bettered by the small amounts which may be used in addition to the minimum amount of approximately .5%. The alloy has many useful applications as previously recited and also may be used in many other instances not mentioned, particularly where a resistance to wear is desirable, for example, on the lips or teeth of steam shovel buckets handling rock. The hardness of the alloy approaching

substantially that of the sapphire, is such that the usual abrasive action of rock does not affect it. The intimate bond of the chromium, molybdenum and iron with the metal of the base upon which the alloy is deposited provides complete assurance against separation therefrom.

I claim:

1. A strong, tough and abrasive resistant alloy adapted to be meltably deposited upon a ferrous base consisting of chromium between 25 and 33%, molybdenum between 1.5 and 5%, copper between 1 and 3%, manganese between 0.5 and 2%, titanium between 0.3 and 1.5% with carbon between 3 to 3.25% and silicon between 0.7 to 1.3%, the balance being of iron with negligible quantities of the usual impurities.

2. An alloy of the class and for the purposes described composed of chromium approximately 25 to 33% molybdenum between 1.5 and 5%, copper between 1 to 3%, titanium between 0.3 to 1.5% with carbon approximating 3% and silicon 0.7 to 1.3%, the balance being of iron with the usual negligible quantities of impurities controlled by the use of manganese in the alloy of approximately 0.5%.

3. An alloy having the properties and for the purposes described composed of chromium between 25 to 33%, molybdenum, 1.5 to 5%, copper 1 to 3%, with carbon between 3 and 3.25%, and silicon between 0.7 and 1.3%, the remainder being iron.

4. An alloy in which the main ingredient is iron and which contains approximately 30% chromium, 3% molybdenum, 2% copper, 1% titanium, 1.5% manganese, 3% carbon and 1% silicon, said iron having the usual negligible phosphorus and sulphur impurities.

WILLIAM C. McLOTT.